



US005906891A

# United States Patent [19]

Shida et al.

[11] Patent Number: **5,906,891**  
[45] Date of Patent: **May 25, 1999**

[54] **ORIENTED POLYAMIDE FIBER AND PROCESS FOR PRODUCING SAME**

[75] Inventors: **Takatoshi Shida; Makoto Takahashi; Masahiro Harada**, all of Kanagawa-ken, Japan

[73] Assignee: **Mitsubishi Gas Chemical Company, Inc.**, Tokyo, Japan

[21] Appl. No.: **09/088,835**

[22] Filed: **Jun. 2, 1998**

## Related U.S. Application Data

[63] Continuation-in-part of application No. 08/762,100, Dec. 9, 1996.

## Foreign Application Priority Data

Dec. 26, 1995 [JP] Japan ..... 7-338981

[51] Int. Cl.<sup>6</sup> ..... D02G 3/00; B29C 47/06

[52] U.S. Cl. ..... 428/364; 428/395; 264/172.18

[58] Field of Search ..... 428/364, 395; 528/347, 310, 322, 335, 336, 264/172.18

## References Cited

### U.S. PATENT DOCUMENTS

- |           |         |                               |
|-----------|---------|-------------------------------|
| 3,629,053 | 12/1971 | Kimura .                      |
| 3,642,565 | 2/1972  | Ogata et al. .                |
| 3,968,071 | 7/1976  | Miyamoto .                    |
| 4,128,599 | 12/1978 | Thomas et al. .               |
| 4,337,179 | 6/1982  | Ueto et al. .                 |
| 4,339,555 | 7/1982  | Ohmura et al. .               |
| 4,433,136 | 2/1984  | Miyamoto et al. ..... 528/347 |
| 4,849,476 | 7/1989  | Mashita et al. .              |
| 4,921,932 | 5/1990  | Tumura et al. .               |
| 5,349,044 | 9/1994  | Liu et al. .                  |
| 5,587,447 | 12/1996 | Harada et al. .               |

## FOREIGN PATENT DOCUMENTS

475 720 3/1992 European Pat. Off. .

## OTHER PUBLICATIONS

Derwent Publications Ltd., London, GB, AN 94-364092, Oct. 11, 1994 of JP 6287807, Mitsubishi Gas Chem. Co.

Primary Examiner—Newton Edwards  
Attorney, Agent, or Firm—Frishauf, Holtz, Goodman, Langer & Chick, P.C.

## ABSTRACT

An oriented polyamide fiber which comprises at least 20% by weight of a crystalline polyamide copolymer (A) produced by polymerizing at least one diamine monomer containing at least 70 mol % m-xylylenediamine and at least one dicarboxylic acid monomer containing at least 70 mol % adipic acid. The oriented polyamide fiber having a Young's modulus of at least 400 kgf/mm<sup>2</sup>, a loop strength of at least 4.5 gf/D, a knot tensile strength of at least 3.5 gf/D and a roundness of from 97 to 100%. A process for producing the oriented polyamide fiber which comprises melting a polyamide resin comprising the crystalline polyamide copolymer (A); spinning the molten resin through a spinneret; pulling the spun product into a coolant bath disposed beneath the face of the spinneret to produce non-oriented fiber to a draw ratio of 2.5 to 8.0 at a temperature not lower than the Tg of the polyamide and not higher than the melting point of the polyamide, wherein the draft ratio is 1.0 to 3.0, and the temperature of the coolant bath (T) satisfies the relational expression: Tg-30≤T≤Tg+10 (°C.). The oriented polyamide fiber can be used in sporting goods and industrial materials such as strings for a racket, rubber reinforcing materials and filter cloth materials for paper making, by virtue of its high strength, modulus of elasticity and roundness.

**15 Claims, No Drawings**

## ORIENTED POLYAMIDE FIBER AND PROCESS FOR PRODUCING SAME

This application is a continuation-in-part application of application Ser. No. 08/762,100, filed Dec. 9, 1996, now abandoned, the entire contents of which are hereby incorporated by reference.

### BACKGROUND OF THE INVENTION

#### 1. Field of the Invention

The present invention relates to oriented polyamide fiber which has a high strength, modulus of elasticity and roundness and which is useful for use in sporting goods such as strings for a racket, in industrial materials such as a rubber reinforcing material and a filter cloth material for paper making and so forth; and a process for producing said polyamide fiber.

#### 2. Description of the Related Arts

Polyamide fiber is generally employed in sporting goods such as strings for a racket, in industrial materials such as a rubber reinforcing material and a filter cloth material for paper making and so forth. In the above-mentioned purposes of use, the polyamide fiber as the construction material is required to be imparted with sufficient modulus of elasticity, that is, Young's modulus and also sufficient mechanical strength including loop strength and knot tensile strength. Moreover in said purposes of use, the polyamide fiber is required to be high in its roundness in the case where a final product made from the fiber is put into practical use, or in the case of secondary processing.

Specifically, when the polyamide fiber is low in its roundness, it will bring about such problems that it is hard to pass the fiber through a clearance or an opening of an accurately processed article, thus lowering the adaptability thereof to machinery and equipment for secondary processing and that the shape of its product after secondary, processing is not uniformized.

A polyamide having repeated units of amide bond which is obtained from m-xylylenediamine and an aliphatic dicarboxylic acid (for example, a polyamide obtained from m-xylylenediamine and adipic acid, hereinafter sometimes referred to as "polyamide MXD6") is expected to find applications in the above-mentioned purpose of use, since it is characterized by its high strength, high Young's modulus and the like as compared with the conventional polyamide 6 and polyamide 66. However, the polyamide MXD6 fiber having high roundness can not be produced with conventional spinning methods, which becomes an obstacle to its practical application.

In more detail, a melt spinning method is usually applied to the production of the polyamide fiber which is employed in sporting goods such as strings for a racket, in industrial materials such as a rubber reinforcing material and a filter cloth material for paper making and so forth. Specifically there is adopted to the production, a spinning method in which a polyamide resin is molten with a single-screw or twin-screw extruder, the molten resin is spun through a spinneret, the spun product is pulled in a coolant bath placed beneath the face of the spinneret to produce non-oriented fiber, and thereafter the non-oriented fiber is oriented. For example, in the case of polyamide 6 or polyamide 66, by the use of non-oriented fiber in which crystallization is suppressed by setting the temperature of a coolant bath lower than the glass transition temperature (Tg) of the polyamide by at least 30° C., it is facilitated to carry out orientation procedures while preserving the roundness of the non-

oriented fiber, whereby the roundness of the fiber is enhanced. The above-mentioned method is exclusively adopted for the purpose of enhancing the roundness of fiber.

On the other hand, in the case of a polyamide containing polyamide MXD6, the Tg of the polyamide MXD6 is remarkably high as compared with that of polyamide 6 or polyamide 66. Therefore, solidification of the non-oriented fiber due to quenching rapidly takes place at a cooling temperature in the conventional melt spinning method for polyamide and at the same time, the resistance in a cooling vessel between the non-oriented fiber and the coolant, and the vibration of the fiber at the time of pulling the fiber in the bath bring about fiber swinging because of the high modulus of elasticity inherent to the polyamide MXD6, whereby the fiber swinging is likely to be transferred to the molten portion of the fiber with a lower strength thus causing a decrease in fiber roundness as well as diametral unevenness of fiber. For this reason, it has heretofore been extremely difficult to steadily and continuously produce a polyamide MXD6-containing polyamide fiber with high roundness.

### SUMMARY OF THE INVENTION

The present invention has been accomplished under the above-described circumstances. Specifically, the object of the present invention is to provide oriented polyamide fiber which has a high strength, modulus of elasticity and roundness and contains polyamide MXD6, and also a process capable of steadily and continuously producing the same through a conventional melt spinning method.

As a result of intensive research and investigation made by the present inventors for the purpose of achieving the aforesigned object, it has been found that the above-mentioned problems are solved by carrying out the melt spinning under specific conditions. The present invention has been completed on the basis of such finding.

Specifically, the present invention provides:

- (1) an oriented polyamide fiber which comprises a crystalline polyamide copolymer (A) (preferably in an amount of 20% by weight) produced by polymerizing at least one diamine monomer consisting essentially of at least 70 mol % m-xylylenediamine and at least one dicarboxylic acid monomer consisting essentially of at least 70 mol % adipic acid, the oriented polymer has a Young's modulus of at least 400 kgf/mm<sup>2</sup>, a loop strength of at least 4.5 gf/D, a knot tensile strength of at least 3.5 gf/D and a roundness in the range of from 97 to 100%;
- (2) the oriented polyamide fiber as set forth in the preceding item (1) which further comprises at most 80% by weight of a (B) crystalline polyamide other than the crystalline polyamide copolymer (A);
- (3) a process for producing an oriented polyamide fiber which comprises the steps of melting a polyamide resin comprising a crystalline polyamide copolymer (A) (preferably in an amount of 20% by weight) produced by polymerizing at least one diamine monomer containing at least 70 mol % m-xylylenediamine and at least one dicarboxylic acid monomer containing at least 70 mol % adipic acid, by the use of a single-screw or twin-screw extruder; spinning the molten resin through a spinneret; pulling the spun product into a coolant bath placed beneath the face of the spinneret to produce non-oriented fiber; and thereafter orienting the non-oriented fiber to a draw ratio of from 2.5 to 8.0 under the temperature conditions of not lower than the glass transition temperature (Tg) of said crystalline polyamide copolymer and not higher than the melting point thereof, wherein the ratio of

the cross-sectional area of the spinneret for a spinning machine (AD) to the cross-sectional area of the non-oriented fiber formed by cooling the product spun by and discharged from the spinning machine in a coolant bath (AM), (AD/AM) (hereinafter referred to as "draft ratio") is in the range of from 1.0 to 3.0, and the temperature of the coolant bath into which the fiber spun by and discharged from the spinning machine is pulled via an air layer made to intervene between a discharge port of the molten resin for the spinning machine and the surface of the coolant bath for cooling the molten resin (T) is in the range satisfying the following relational expression:

$$T_{g-30} \leq T \leq T_{g+10} (\text{°C.});$$

and

(4) the process for producing an oriented polyamide fiber as set forth in the preceding item (3) wherein the polyamide resin is a polyamide resin comprising at least 20% by weight of the crystalline polyamide copolymer (A) and which further comprises at most 80% by weight of a (B) crystalline polyamide other than the crystalline polyamide copolymer (A).

#### DESCRIPTION OF THE PREFERRED EMBODIMENTS

The crystalline polyamide copolymer (A) to be used in the present invention is produced by polymerizing at least one diamine monomer containing at least 70 mol % m-xylylenediamine and at least one dicarboxylic acid monomer containing at least 70 mol % adipic acid.

In the case where the crystalline polyamide copolymer (A) is produced by polymerizing a diamine containing less than 70 mol % m-xylylenediamine and a dicarboxylic acid monomer containing less than 70 mol % adipic acid, the polyamide fiber finally formed therefrom does not possess characteristics such as high strength and high Young's modulus.

Illustrative examples of the unit other than m-xylylenediamine as the diamine component (monomer), used within an amount of 30 mol % or less, to form the "crystalline polyamide copolymer (A)", include aliphatic diamines such as tetramethylene diamine, pentamethylene diamine, octamethylene diamine and non-amethylene diamine; aromatic diamines such as paraphenylenediamine; alicyclic diamines such as 1,3-bisaminomethyl cyclohexane and 1,4-bisaminomethyl cyclohexane; and the like.

Illustrative examples of the unit other than adipic acid as the dicarboxylic acid component (monomer), used within an amount of 30 mol % or less, to form the "crystalline polyamide copolymer (A)" include aliphatic dicarboxylic acids such as succinic acid, glutaric acid, pimelic acid, suberic acid, azelaic acid, sebacic acid, undecane diacid and dodecane diacid; aromatic dicarboxylic acids such as terephthalic acid, isophthalic acid and 2,6-naphthalene dicarboxylic acid; and the like.

The oriented polyamide to be used in the present invention may contain a (B) crystalline polyamide other than the crystalline polyamide copolymer (A). A variety of polyamides are available as the crystalline polyamide (B) other than the crystalline polyamide copolymer (A) and are specifically exemplified by polyamide 6, polyamide 66, polyamide 6/66 (a copolymer of polyamide 6 component and polyamide 66 component), polyamide 610, polyamide 612, polyamide 11, polyamide 12 and a mixture thereof. Of these,

polyamide 6, polyamide 66 and polyamide 6/66 are preferably used in the present invention. By the use of any of the above-exemplified polyamide resins, it is made easy to regulate the physical properties of the objective fiber such as strength and elongation percentage by adjusting the conditions at the time of melt extrusion.

It is necessary that the oriented polyamide fiber according to the present invention contains at least 20% by weight of the aforesaid crystalline polyamide copolymer (A). In the case where the blending proportion of the crystalline polyamide copolymer (A) in the fiber is less than 20% by weight, it is difficult to obtain the characteristics inherent in polyamide MXD6 such as high strength, high modulus of elasticity and crystallization rate facilitating the spinning be reflected upon the physical properties of the objective polyamide fiber. It is also preferable that the blending proportion of the crystalline polyamide (B) be at most 80% by weight.

The oriented polyamide fiber according to the present invention has a Young's modulus of at least 400 kgf/mm<sup>2</sup>, preferably at least 500 kgf/mm<sup>2</sup>. In the case where the oriented polyamide fiber having a Young's modulus of less than 400 kgf/mm<sup>2</sup> is used for strings for a racket, a rubber reinforcing material or a filter cloth material for paper making, deformation takes place, thus depriving the fiber product of commodity value.

In addition, the oriented polyamide fiber according to the present invention has a loop strength of at least 4.5 gf/D, preferably at least 5.0 gf/D. In the case where the oriented polyamide fiber having a loop strength of less than 4.5 gf/D is used for strings for a racket, breaking of the strings takes place at the bending portion thereof at the time of being attached to the racket, thus depriving the fiber product of commodity value; and besides when it is used for a filter cloth material for paper making, since the filter cloth material is attached to a roll for a paper machine by a method wherein part of filter cloth fiber is bent and the filter cloth material is connected to the roll by passing core threads through the resultant bending part, breaking of the cloth material takes place at the connecting portion, thereby depriving the filter cloth of commodity value.

Moreover, the oriented polyamide fiber according to the present invention has a knot tensile strength of at least 3.5 gf/D, preferably at least 4.0 gf/D. In the case where the oriented polyamide fiber having a knot tensile strength of less than 3.5 gf/D is used for strings for a racket, breaking of the strings takes place at the knots thereof at the time of being mounted on the racket, whereby the commodity value of the strings is lost.

The present invention also relates to a process for producing oriented polyamide fiber which comprises the steps of melting a polyamide resin comprising at least 20% by weight of the crystalline polyamide copolymer (A) produced by polymerizing at least one diamine monomer containing at least 70 mol % of m-xylylenediamine and at least one dicarboxylic acid monomer containing at least 70 mol % of adipic acid by the use of a single-screw or twin-screw extruder; spinning the molten resin through a spinneret; pulling the spun product into a coolant bath placed beneath the face of the spinneret to produce non-oriented fiber; and thereafter orienting the non-oriented fiber to a draw ratio of from 2.5 to 8.0 under the temperature conditions of not lower than T<sub>g</sub> of said polyamide and not higher than the melting point thereof.

In particular, with regard to the process according to the present invention, the draft ratio, that is, the ratio of the cross-sectional area of the spinneret for a spinning machine

(AD) to the cross-sectional area of the non-oriented fiber formed by cooling the product spun by and discharged from the machine in a coolant bath (AM), (AD/AM) is 1.0 to 3.0, preferably 1.0 to 2.5. A draft ratio of less than 1.0 in the aforesaid process makes it difficult to actually produce non-oriented fiber, whereas that of more than 3.0 makes it difficult to produce polyamide fiber having high roundness, since the influence of the extruding and cooling conditions exerted upon the non-oriented fiber is amplified. In the process according to the present invention, the AM, that is, the cross-sectional area of the non-oriented fiber formed by cooling the product spun by and discharged from the machine in a coolant bath is specified by the following formula:

$$AM(\text{cm}^2)G/(L \times \rho)$$

wherein G stands for the weight in g of the non-oriented fiber having a density of  $\rho$  in  $\text{g/cm}^2$  and a length of L in cm.

It is necessary in the process according to the present invention to make an air layer intervene between a discharge port of the molten resin for the spinning machine and the surface of the coolant bath for cooling the molten resin for the purpose of preventing the fiber from being quenched. Nonexistence of an air layer therebetween brings about such troubles as fiber swinging due to coolant boiling at the time when the molten resin is brought into contact with the coolant and the generation of vacuum foams due to quenched fiber.

In view of the foregoing, it is preferable that the thickness of the aforesaid air layer, namely the distance between the discharge port of the molten resin for the spinning machine and the surface of the coolant bath for cooling the molten resin (hereinafter referred to as "air gap") be at least 10 mm from the practical point of view. The air layer, when being unreasonably thick, will make it difficult to produce polyamide fiber having high roundness because of the drawdown, etc. of the molten resin. For this reason, the air gap is preferably 150 mm or less from the practical viewpoint. In the process of the present invention, the air gap is more preferably from 10 to 110 mm.

It is required, in the process according to the present invention that the temperature of the coolant bath (T) into which the polyamide fiber discharged from the spinning machine is pulled be in the temperature range satisfying the following relational expression:

$$Tg-30 \leq T \leq Tg+10 (\text{ }^{\circ}\text{C.})$$

which specifies the relationship between  $Tg$  of the polyamide resin and T. The temperature of the coolant bath (coolant temperature), when being lower than  $Tg-30$  ( $^{\circ}\text{C.}$ ), will give rise to trouble such as the generation of voids due to the difference in temperature between the surface of the non-oriented fiber and the inside thereof or due to the fiber quenching. On the other hand, the temperature thereof, when being higher than  $Tg+10$  ( $^{\circ}\text{C.}$ ), will bring about such troubles as the collapse of the non-oriented fiber due to insufficient cooling and difficulty in orientation due to the crystallization of the non-oriented fiber.

In the case of using a material formed by blending a plurality (N) of polyamide resins,  $Tg$  of the resultant blend to be adopted in the present invention is defined by the formula

$$Tg(\text{ }^{\circ}\text{C.}) = a \times TgA + b \times TgB + c \times TgC + \dots + n \times TgN$$

wherein a, b, c, . . . n each stand for the volumetric fraction of the component A, B, C, . . . N, and  $TgA$ ,  $TgB$ ,  $TgC$ , . . .  $TgN$  each represent  $Tg$  of the component A, B, C, . . . N.

In the process according to the present invention, it is made possible to produce polyamide fiber having high roundness by setting the coolant temperature at a higher level than that of the conventional general spinning conditions and also to dispense with a coolant cooler which has heretofore been necessary.

The crystalline polyamide copolymer (A) produced by polymerizing at least one diamine monomer containing at least 70 mol % m-xylylenediamine and at least one dicarboxylic acid monomer containing at least 70 mol % adipic acid, which polyamide is produced in the production process according to the present invention, is the polyamide which is contained in the oriented polyamide fiber according to the present invention. The single-screw or twin-screw extruder to be used for melt spinning in the process of the invention can be optionally selected for use from a variety of extruders for conventional application. Mixing of the crystalline polyamide copolymer and the crystalline polyamide other than (A), namely the crystalline polyamide (B), to be used in the present invention can be carried out by any of a method generally referred to as a "dry blending method" in which, for example, solid materials such as pellets as such are fed in an extruder under mixing, and a method generally referred to as a "melt blending method" in which solid materials are once melt extruded together to pelletize the same and the resultant pellets are used as the starting raw material. As described hereinbefore, the present invention is concerned with a process for producing oriented polyamide fiber oriented to a draft ratio of from 2.5 to 8.0 at a temperature not lower than  $Tg$  of the polyamide resin and not higher than the melting point thereof.

Likewise, the present invention pertains to oriented polyamide fiber having a roundness in the range of from 97 to 100% and a process for producing the same. The value of roundness (%) is defined by the following formula, and the closer the value to 100%, the closer the cross-sectional shape of a filament to a true circle.

$$\text{Roundness \%} = (1/n) \sum_{i=1}^n [(RSi / RMi) \times 100]$$

wherein  $RSi$  (mm) is the smallest fiber diameter at the i'th point among the measuring points of n numbers, and  $RMi$  (mm) is the median fiber diameter at the i'th point among the measuring points of n numbers.

In the case where the roundness of the polyamide fiber is less than 97%, a definite shape is not obtained, for example, in the multi-layer structural fibers such as a modern tennis gut and woven or nonwoven fabric such as a filter cloth material for paper making, thus causing the loss of their commodity values; and besides, there are brought about such troubles as difficulty in passing the fiber through a clearance or an opening of a precisely processed article, and low adaptability to machinery and equipment for secondary processing.

It is possible according to the present invention to produce oriented polyamide fiber having a diameter after final orientation of 0.05 to 2 mm, preferably 0.1 to 1.5 mm.

The polyamide resin to be used in the present invention may be incorporated as necessary with an inorganic or organic compound such as thermal-age resister, color preventive agent, crosslinking preventive agent, weatherability improver, ultraviolet absorber, pigment, antistatic agent and flame retardant, each alone or in optional combination with one another.

The usable coolant in the process according to the present invention is exemplified by water, glycerol, liquid paraffin, silicone oil, hydrocarbon series oil, polyethylene glycol and diethylene glycol.

The oriented polyamide fiber obtained through the present invention is useful for use in sporting goods such as strings for a racket and in industrial materials such as a rubber reinforcing material and a filter cloth material for paper making and so forth by virtue of its high strength, modulus of elasticity and roundness.

In the following, the present invention will be described in more detail with reference to comparative examples and working examples, which however, shall not restrict the present invention thereto. Measurements were made of the strength and Young's modulus of the oriented fiber according to JIS L 1013 "Testing method for chemically synthesized filament fiber", and of the diameter of the oriented fiber by measuring a smallest diameter and a largest diameter at 100 numbers of arbitrary points with a spacing of 10 cm each.

In the following Tables 1, 2 and 3, m-xylylenediamine, p-xylylenediamine, hexamethylenediamine, adipic acid, terephthalic acid, sebacic acid and polyamide 6, are abbreviated as MXDA, PXDA, HMDA, AA, TA, SA and N-6, respectively.

#### EXAMPLE 1

A polyamide copolymer comprising 100 mol % of m-xylylenediamine as a diamine component, and 80 mol % of adipic acid and 20 mol % of terephthalic acid as a dicarboxylic acid component was molten by the use of a single-screw extruder, spun through a spinneret at a temperature of 260° C., pulled into a water bath at 80° C. under the conditions including a draft ratio of 2.3 and an air gap of 100 mm, and continuously oriented without temporary winding.

The orientation was put into practice by two stages of orientation and a single stage of heat setting. There were used as orientation means, a warm water bath at 90° C. in the first stage orientation region, a dry hot air bath at 220° C. in the second stage orientation region and a dry hot air bath at 280° C. in the heat setting region. As the orientation conditions, the overall draw ratio, the second stage draw ratio and the relaxation ratio were set on 5.0, 1.2 and 5%, respectively. By the above-mentioned procedures, there was produced polyamide copolymer single fiber at a production velocity of 75 m/min. The fiber diameter and roundness of the polyamide copolymer fiber thus obtained are given in Table 1.

#### EXAMPLE 2

The procedure in Example 1 was repeated except that a polyamide copolymer comprising 100 mol % of m-xylylenediamine as a diamine component and 80 mol % of adipic acid and 20 mol % of sebacic acid as a dicarboxylic acid component was molten by the use of a single-screw extruder and pulled into a water bath at 60° C. The fiber diameter and roundness of the polyamide copolymer fiber thus obtained are given in Table 1.

#### EXAMPLE 3

The procedure in Example 1 was repeated except that a polyamide copolymer comprising 80 mol % of m-xylylenediamine and 20 mol % of p-xylylenediamine as a diamine component and 100 mol % of adipic acid as a dicarboxylic acid component was molten by the use of a

single-screw extruder and pulled into a water bath at 70° C. The fiber diameter and roundness of the polyamide copolymer fiber thus obtained are given in Table 1.

#### EXAMPLE 4

The procedure in Example 1 was repeated except that a polyamide copolymer comprising 80 mol % of m-xylylenediamine and 20 mol % of hexamethylenediamine as a diamine component and 100 mol % of adipic acid as a dicarboxylic acid component was molten by the use of a single-screw extruder and pulled into a water bath at 60° C. The fiber diameter and roundness of the polyamide copolymer fiber thus obtained are given in Table 2.

#### EXAMPLE 5

The procedure in Example 1 was repeated except that a polyamide copolymer comprising 100 mol % of m-xylylenediamine as a diamine component, and 80 mol % of adipic acid and 20 mol % of terephthalic acid as a dicarboxylic acid component and polyamide 6 (produced by Ube Industries, Ltd. under the trade name "1011FB") were dry blended in a ratio by weight of 30/70, molten by the use of a single-screw extruder, and pulled into a water bath at 30° C. The fiber diameter and roundness of the polyamide copolymer fiber thus obtained are given in Table 2.

#### EXAMPLE 6

The procedure in Example 1 was repeated except that a polyamide copolymer comprising 80 mol % of m-xylylenediamine and 20 mol % of p-xylylenediamine as a diamine component and 100 mol % of adipic acid as a dicarboxylic acid component and the same polyamide 6 as used in Example 5 were dry blended in a ratio by weight of 30/70, molten by the use of a single-screw extruder, and pulled into a water bath at 30° C. The fiber diameter and roundness of the polyamide copolymer fiber thus obtained are given in Table 2.

#### EXAMPLE 7

The procedure in Example 1 was repeated except that a polyamide copolymer comprising 70 mol % of m-xylylenediamine and 30 mol % of p-xylylenediamine as a diamine component and 70 mol % of adipic acid and 30 mol % of terephthalic acid as a dicarboxylic acid component and the same polyamide 6 as used in Example 5 were dry blended in a ratio by weight of 30/70, molten by the use of a single-screw extruder, and pulled into a water bath at 30° C. The fiber diameter and roundness of the polyamide copolymer fiber thus obtained are given in Table 3.

#### COMPARATIVE EXAMPLE 1

The procedure in Example 1 was repeated except that a polyamide copolymer comprising 100 mol % of m-xylylenediamine as a diamine component, and 50 mol % of adipic acid and 50 mol % of sebacic acid as a dicarboxylic acid component was molten by the use of a single-screw extruder and pulled into a water bath at 60° C. The fiber diameter and roundness of the polyamide copolymer fiber thus obtained are given in Table 3.

#### COMPARATIVE EXAMPLE 2

The procedure in Example 1 was repeated except that a polyamide copolymer comprising 50 mol % of m-xylylenediamine and 50 mol % of hexamethylenediamine

as a diamine component, and 100 mol % of adipic acid as a dicarboxylic acid component was molten by the use of a single-screw extruder and pulled into a water bath at 60° C. The fiber diameter and roundness of the polyamide copolymer fiber thus obtained are given in Table 3.

TABLE 1

| Number of Example                      | Example 1          | Example 2          | Example 3 |
|----------------------------------------|--------------------|--------------------|-----------|
| <u>Resin used</u>                      |                    |                    |           |
| Diamine (mol %)                        | MXDA : 100         | MXDA : 100         | MXDA : 80 |
| Dicarboxylic acid (mol %)              | AA : 80<br>TA : 20 | AA : 80<br>SA : 20 | AA : 100  |
| N-6 blending proportion                | 0                  | 0                  | 0         |
| Draft ratio                            | 2.3                | 2.3                | 2.4       |
| Air gap (mm)                           | 100                | 100                | 100       |
| Coolant temperature (° C.)             | 80                 | 60                 | 70        |
| Draw ratio                             | 5.0                | 5.0                | 5.0       |
| Diameter of oriented fiber (mm)        |                    |                    |           |
| Minimum small diameter                 | 0.47               | 0.47               | 0.47      |
| Maximum large diameter                 | 0.48               | 0.48               | 0.48      |
| Median fiber diameter                  | 0.48               | 0.48               | 0.48      |
| Roundness (%)                          | 99.4               | 99.4               | 99.3      |
| Young's modulus (kgf/mm <sup>2</sup> ) | 830                | 740                | 850       |
| Tensile strength (gf/D)                | 6.2                | 6.0                | 6.0       |
| Knot tensile strength (gf/D)           | 4.1                | 4.6                | 4.4       |
| Loop strength (gf/D)                   | 4.9                | 5.4                | 5.0       |

TABLE 2

| Number of Example                      | Example 4              | Example 5          | Example 6              |
|----------------------------------------|------------------------|--------------------|------------------------|
| <u>Resin used</u>                      |                        |                    |                        |
| Diamine                                | MXDA : 80<br>HMDA : 20 | MXD6 : 100         | MXD6 : 80<br>PXDA : 20 |
| Dicarboxylic acid                      | AA : 100               | AA : 80<br>TA : 20 | AA : 100               |
| N-6 blending proportion                | 0                      | 70                 | 70                     |
| Draft ratio                            | 2.3                    | 2.3                | 2.4                    |
| Air gap (mm)                           | 100                    | 100                | 100                    |
| Coolant temperature (° C.)             | 60                     | 30                 | 30                     |
| Draw ratio                             | 5.0                    | 5.0                | 5.0                    |
| Diameter of oriented fiber (mm)        |                        |                    |                        |
| Minimum small diameter                 | 0.47                   | 0.47               | 0.47                   |
| Maximum large diameter                 | 0.48                   | 0.48               | 0.48                   |
| Median fiber diameter                  | 0.48                   | 0.48               | 0.48                   |
| Roundness (%)                          | 99.4                   | 99.4               | 99.3                   |
| Young's modulus (kgf/mm <sup>2</sup> ) | 730                    | 540                | 550                    |
| Tensile strength (gf/D)                | 6.2                    | 6.0                | 6.0                    |
| Knot tensile strength (gf/D)           | 4.1                    | 4.6                | 4.4                    |
| Loop strength (gf/D)                   | 4.9                    | 8.0                | 8.4                    |

TABLE 3

| Number of Example          | Example 7              | Comp. Example 1    | Comp. Example 2        |
|----------------------------|------------------------|--------------------|------------------------|
| <u>Resin used</u>          |                        |                    |                        |
| Diamine                    | MXDA : 70<br>PXDA : 30 | MXDA : 100         | MXDA : 50<br>HMDA : 50 |
| Dicarboxylic acid          | AA : 70<br>TA : 30     | AA : 50<br>SA : 50 | AA : 100               |
| N-6 blending proportion    | 0                      | 0                  | 0                      |
| Draft ratio                | 2.4                    | 2.3                | 2.4                    |
| Air gap (mm)               | 100                    | 100                | 100                    |
| Coolant temperature (° C.) | 30                     | 60                 | 50                     |
| Draw ratio                 | 5.0                    | 5.0                | 5.0                    |

TABLE 3-continued

| Number of Example                      | Example 7                              | Comp. Example 1 | Comp. Example 2 |
|----------------------------------------|----------------------------------------|-----------------|-----------------|
| <u>Diameter of oriented fiber (mm)</u> |                                        |                 |                 |
| 10                                     | Minimum small diameter                 | 0.47            | 0.47            |
|                                        | Maximum large diameter                 | 0.48            | 0.48            |
|                                        | Median fiber diameter                  | 0.48            | 0.48            |
|                                        | Roundness (%)                          | 99.3            | 99.4            |
|                                        | Young's modulus (kgf/mm <sup>2</sup> ) | 550             | 600             |
|                                        | Tensile strength (gf/D)                | 6.0             | 5.0             |
| 15                                     | Knot tensile strength (gf/D)           | 4.4             | 3.6             |
|                                        | Loop strength (gf/D)                   | 8.4             | 4.0             |

What is claimed is:

- An oriented polyamide fiber which comprises a crystalline polyamide copolymer (A) produced by polymerizing at least one diamine monomer and at least one dicarboxylic acid monomer, said diamine monomer consisting essentially of at least 70 mol % of m-xylylenediamine, said dicarboxylic acid monomer consisting essentially of at least 70 mol % of adipic acid, said oriented polyamide fiber having a Young's modulus of at least 400 kgf/mm<sup>2</sup>, a loop strength of at least 4.5 gf/D, a knot tensile strength of at least 3.5 gf/D and a roundness of 97 to 100%.
- The oriented polyamide fiber according to claim 1, which further comprises at most 80% by weight of a (B) crystalline polyamide other than the crystalline polyamide copolymer (A).
- The oriented polyamide fiber according to claim 2, wherein the crystalline polyamide (B) is at least one member selected from the group consisting of polyamide 6, polyamide 66 and a copolymer of a polyamide 6 component and a polyamide 66 component.
- The oriented polyamide fiber according to claim 1, wherein the diamine monomer contains 30 mol % or less of a diamine selected from the group consisting of an aliphatic diamine, an aromatic diamine and an alicyclic diamine.
- The oriented polyamide fiber according to claim 1, wherein the diamine monomer contains 30 mol % or less of a diamine selected from the group consisting of tetramethylene diamine, pentamethylene diamine, octamethylene diamine, nonamethylene diamine, paraphenylenediamine, 1,3-bisaminomethyl cyclohexane and 1,4-bisaminomethyl cyclohexane.
- The oriented polyamide fiber according to claim 1, wherein the dicarboxylic acid monomer contains 30 mol % or less of a dicarboxylic acid selected from the group consisting of an aliphatic dicarboxylic acid, and an aromatic dicarboxylic acid.
- The oriented polyamide fiber according to claim 1, wherein the dicarboxylic acid monomer contains 30 mol % or less of a dicarboxylic acid selected from the group consisting of succinic acid, glutaric acid, pimelic acid, suberic acid, azelaic acid, sebaic acid, undecane diacid, dodecane diacid, terephthalic acid, isophthalic acid and 2,6-naphthalene dicarboxylic acid.
- The oriented polyamide fiber according to claim 5, wherein the dicarboxylic acid monomer contains 30 mol % or less of a dicarboxylic acid selected from the group consisting of succinic acid, glutaric acid, pimelic acid, suberic acid, azelaic acid, sebaic acid, undecane diacid, dodecane diacid, terephthalic acid, isophthalic acid and 2,6-naphthalene dicarboxylic acid.
- The oriented polyamide fiber according to claim 1, wherein the Young's modulus is at least 500 kgf/mm<sup>2</sup>, the

**11**

loop strength is at least 5.0 gf/D, and the knot tensile strength is at least 4.0 gf/D.

**10.** The oriented polyamide fiber according to claim **8**, wherein the Young's modulus is at least 500 kgf/mm<sup>2</sup>, the loop strength is at least 5.0 gf/D, and the knot tensile strength is at least 4.0 gf/D.

**11.** A process for producing the oriented polyamide fiber according to claim **1** having a Young's modulus of at least 400 kgf/mm<sup>2</sup>, a loop strength of at least 4.5 gf/D, a knot strength of at least 3.5 gf/D and a roundness of 97 to 100%, which comprises melting a polyamide resin comprising a crystalline polyamide copolymer (A) produced by polymerizing (i) at least one diamine monomer containing at least 70 mol % m-xylylenediamine and (ii), at least one dicarboxylic acid monomer containing at least 70 mol % adipic acid, by the use of a single-screw or twin-screw extruder; spinning the molten resin through a spinneret; pulling the spun product into a coolant bath disposed beneath the face of the spinneret to produce non-oriented fiber; and thereafter orienting the non-oriented fiber to a draw ratio of from 2.5 to 8.0 at the temperature conditions of not lower than the glass transition temperature (Tg) of said polyamide and not higher than the melting point of said polyamide, wherein the ratio of the cross-sectional area of the spinneret for a spinning machine (AD) to the cross-sectional area of the non-oriented fiber formed by cooling the product spun by and discharged from the spinning machine in a coolant bath (AM), (AD/AM) is 1.0 to 3.0, and the temperature of the coolant bath into which the fiber spun by and discharged from the

**12**

spinning machine is pulled via an air layer made to intervene between a discharge port of the molten resin for the spinning machine and the surface of the coolant bath for cooling the molten resin (T) is in the range satisfying the relational expression

$$T_g-30 \leq T \leq T_g+10 (\text{°C.})$$

**12.** The process for producing oriented polyamide fiber according to claim **11**, wherein the polyamide resin further comprises at most 80% by weight of a crystalline polyamide (B) other than the crystalline polyamide copolymer (A).

**13.** The process for producing oriented polyamide fiber according to claim **12**, wherein the crystalline polyamide (B) is at least one member selected from the group consisting of polyamide 6, polyamide 66 and a copolymer of a polyamide 6 component and a polyamide 66 component.

**14.** The process for producing oriented polyamide fiber according to claim **11**, wherein the distance between the discharge port of the molten resin for the spinning machine and the surface of the coolant bath for cooling the molten resin is 10 to 150 mm.

**15.** The process for producing oriented polyamide fiber according to claim **11**, wherein the crystalline polyamide resin comprises at least 20 wt % of the crystalline polyamide copolymer (A).

\* \* \* \* \*